# EUROPEAN PATENT SPECIFICATION

(11) **EP 2 828 863 B1**
(45) Date of publication and mention of the grant of the patent: **16.09.2020**
(21) Application number: 13764112.2
(22) Date of filing: 19.03.2013
(51) Int. Cl.: H01B 7/08, H01R 13/03, H02G 5/00, H01B 17/62

(54) **BUSBAR**
STROMSCHIENE
BARRE OMNIBUS

(30) Priority: 20.03.2012 AU 2012901127
(43) Date of publication of application: 28.01.2015
(73) Proprietor: Albus Industries Pty Ltd, Maddington Western Australia 6989 (AU)
(72) Inventor: DE LAETER, Richard Lionel, Maddington Western Australia 6109 (AU)
(74) Representative: Wildhack & Jellinek
(86) International application number: PCT/AU2013/000277
(87) International publication number: WO 2013/138853

(56) References cited:
- CN-Y- 201 036 072
- CN-Y- 201 036 072
- US-A- 3 086 888
- FARAHAT ET AL.: 'Effect of Coating Materials on the Electrical Performance of Copper Joints' ELECTRICAL CONTACTS, 1996. PROCEEDINGS OF THE FORTY-SECOND IEEE HOLM CONFERENCE 16 September 1996, CHICAGO, IL, USA, pages 472 - 478, XP032156715

## Description

### FIELD OF THE INVENTION

The present invention relates to a method of manufacturing an apparatus for electrical connection and in particular to a method of manufacturing a pre-insulated busbar for use in an electrical distribution apparatus such as a switch board.

### BACKGROUND

It is known to use a busbar for electrical power distribution in switch boards and other electrical apparatus. A naked busbar typically comprises a plain length of highly conductive metal, such as copper or aluminium, for conducting and distributing electricity.

Busbars are often configured as a flat strip to provide a high surface area to volume ratio which assists in effective heat dissipation. Busbars are often used to conduct dangerous voltages and high currents, in order to protect against accidental electrocution, short circuits or internal arcing faults, insulation of a naked busbar is carried out as an additional step in the assembly of a switch board.

A busbar will often need to be shaped or prepared in some way (i.e. holes drilled) in order for the busbar to fit a particular switch board, electrical apparatus or connection. Prior art busbars are supplied in a naked state and it is not known for a busbar to be insulated prior to shaping or fabricating the busbar.

Known techniques for insulating a naked busbar are carried out after the busbar has been shaped and/or otherwise prepared. US 3086 888 describes a method for isolating a busbar with a specific epoxy resin by dip coating. Further techniques include heat shrink sleeving, PVC (or similar) rigid sleeving or powder coating. Heat shrink sleeving is expensive and prone to becoming fragile and brittle over time. Moreover this method of insulation is time consuming as a naked busbar must first be shaped and assembled into a switchboard, then disassembled, before being reassembled with an insulating heat shrink fitted. PVC sleeving has good mechanical strength and is generally cheaper than heat shrink sleeving however the thickness of the PVC sleeve creates difficulties when fitting a PVC sleeved busbar into a switch board having standard busbar supports. CN 201036072 describes a busbar manufactured by powder coating. Known powder coating techniques requires a naked busbar to be at least partly assembled, then taken apart and the connecting surfaces masked with a heat resistant tape before a powder coating is applied.

The metal materials used in a busbar include copper or aluminium. Both of these materials are reactive to oxygen in the atmosphere whereby a hard oxide layer naturally forms upon a naked metal surface. Oxide layers form quickly and have a high resistance to current flow and interfere with the optimal functioning of a busbar which can lead to failure of connections over time.

It is also known to plate a copper busbar with tin to limit the formation of an oxide layer. In use, an oxide layer on a busbar must be punctured and preferably used with a contact lubricant to reduce electrical resistance when connecting the busbar to other busbars or electrical apparatus.

In Australia the prevalent material used in a busbar is copper. Copper has a high electrical conductivity, good corrosion resistance and is a soft metal that is relatively easy to work with. However, the weight and high cost of copper are factors which are problematic.

Aluminium material is less expensive than copper however the cross sectional area of an aluminium busbar must be around 60% greater than an equivalent copper busbar to achieve the same thermal rating. The oxide layer that forms on an aluminium metal surface is self limiting to around a thickness of 10µm and is electrically resistive causing failure of connections over time. For this reason prior art aluminium busbars must be treated more carefully than is necessary for copper busbars. After shaping and/or preparing a prior art naked aluminium busbar the connecting surfaces are abraded to remove the oxide layer and immediate connection, often using a special contact lubricant to exclude contact with air, is required to avoid the oxide layer reforming. Therefore producing, maintaining or otherwise working with switch boards using known naked aluminium busbars requires additional skills and time consuming measures when compared with a copper busbar equivalent.

The present invention attempts to provide a useful alternative method for manufacturing the aforementioned prior art aluminium and copper busbars.

It is an object of the present invention to provide a method for manufacturing apre-insulated busbar comprising a conductive barrier for limiting oxide layers forming on the busbar.

It is a further object of the present invention to provide a method for manufacturing a pre-insulated busbar enabling good electrical connectivity and corrosion resistance when connected with dissimilar metals.

It is a further object of the present invention to provide a method for manufacturing a pre-insulated aluminium busbar having good electrical connectivity and corrosion resistance when connecting to other busbars or electrical components.

It is a further object of the present invention to provide a method for manufacturing the pre-insulated busbar that comprises an electrically insulating barrier that is selectively removable from the busbar.

It is a yet a further object of the present invention to provide a method for manufacturing the pre-insulated busbar capable of being shaped without compromising the efficacy of the electrical insulation barrier.

It is an object of the present invention to provide a method for manufacturing the pre-insulated busbar enabling safe, simple and fast electrical connections.

### SUMMARY OF THE INVENTION

In accordance with a first aspect of the present invention there is provided a method for manufacturing an insulated busbar for use in electrical distribution, the busbar comprising a metallic body having at least an external surface disposed between peripheral ends, wherein the busbar comprises a substantially electrically insulating barrier covering at least a portion of the external surface for limiting an undesired electrical connection with the exterior surface.

The insulating barrier comprises a plastic surface coating.

The plastic surface coating has ductile properties.

In accordance with a second aspect of the present invention there is provided a method for manufacturing an insulated busbar for use in electrical distribution, the busbar comprising a body having an exterior surface disposed between peripheral ends, wherein the busbar comprises a substantially electrically conductive barrier covering at least a portion of the external surface for limiting an undesired metallic oxide layer forming on the exterior surface.

Preferably the conductive barrier comprises a metallic surface coating.

In accordance with a further aspect of the present invention there is provided a method for manufacturing an insulated busbar for use in electrical distribution having a first portion and a second portion, characterised in that the first portion comprises the conductive barrier and the second portion comprises the insulating barrier.

In a preferred embodiment of the present invention the metallic surface coating comprises nickel material.

The plastic surface coating is applied to the busbar external surface using a powder coating process.

In a preferred embodiment the insulating barrier may be selectively removable from the exterior surface by scoring the plastic surface coating and peeling it away from the exterior surface. Preferably no plastic residue remains on an exposed external surface after the plastic surface coating has been removed.

Preferably the metallic surface coating and the plastic surface coatings limit marking of the busbar through handling.

The metallic surface coating and the plastic surface coating are applied to a busbar prior to a shaping of the busbar in use.

### BRIEF DESCRIPTION OF THE DRAWINGS

The present invention will now be described, by way of example, with reference to the accompanying drawings, in which:
Figure 1 shows an "L" shaped busbar; and
Figure 2 shows a flat busbar.

### DESCRIPTION OF THE PREFERRED EMBODIMENTS

Referring to the Figures, there is shown a busbar 10 comprising a body 12 having an external surface 13 disposed between peripheral ends 6,8. The external surface 13 preferably comprises at least a first planar surface 14 and an opposed second planar surface 16, the first surface 14 and second surface 16 being spaced apart by an edge 18 corresponding to a thickness of the busbar 10.

In the embodiment shown in Figure 1 the busbar has an "L" shaped configured however it is to be understood that the busbar 10 is not limited in shape and may take any particular shape or configuration as desired including a straight flat busbar 10 shown in Figure 2. It is an advantage of the present invention that the busbar is insulated prior to being shaped or bent or otherwise prepared as required for use with a particular electrical connection or electrical distribution apparatus.

It should be understood that the features of the present invention may be applied to a busbar either separately or in combination. Therefore, a busbar 10 manufactured according to the present invention may comprise an insulating barrier alone or together with a conductive barrier.

In one preferred embodiment the busbar 10 comprises an aluminium material which is made from an electrical grade of aluminium having desired characteristics of bendability and mechanical strength. Typically a busbar 10 of aluminium material will comprise Alloy 6101 and a temper T6 giving the following typical material properties:

| | |
|---|---|
| Electrical conductivity: | 57% IACS (International Annealed Copper Standard) |
| Melting range: | approximately 660° C |
| Max. thermal capacity: | 319µΩ mm² |
| Thermal conductivity: | 20.5/25 kgf/mm² |

### Electrically Conductive Barrier

As shown in the figures the busbar 10 is arranged to have a first portion 20 covered by an electrically conductive barrier 22. The conductive barrier 22 comprises a metallic surface coating 22 which is arranged to cover a portion 20 of the external surface 13. Preferably the first portion 20 may comprise a substantial entirety of the external surface 13.

It is to be understood that the metallic surface coating 22 is configured to limit a metallic oxide layer forming on the external surface 13 of the first portion 20 of the busbar 10. The metallic surface coating 22 preferably comprises the element nickel which, when applied in accordance with the present invention has been found to provide the following suitable characteristics:
Good adherence to the aluminium after proper preparation
Low electrical resistance
Compatible with copper, tin, silver and aluminium materials and coatings which are used for connections with the busbar.
Ductile, allowing the busbar to be bent without fracturing or compromising the nickel plated surface.

The metallic surface coating 22 may be applied by any known means but a preferred embodiment of the present invention involves an electrodeposition method.

In accordance with the present invention, a method of providing a metallic surface coating 22 on a busbar 10 made of aluminium material is described below.

### Mounting:

The busbar 10 is suspended on a mounting rack for the pre-treatment and electroplating processes.

### Cleaning:

The busbar 10 is immersed for a period of time in a heated cleaner solution for the removal of surface impurities such as oils, grease or other compounds. Typically the busbar 10 will be immersed in a hot chemical solution for a period of 12 minutes. The chemical solution described for cleaning may comprise a solution of Oxidite C-10 at a temperature of 60°C.

The cleaned busbar 10 is then immersed or spray rinsed in demineralised water.

### Etching:

The portion 20 of the busbar 10 is immersed for a period of time in a heated etching solution for the removal of surface material from the busbar 10. Typically the busbar 10 will be immersed for a period of around 2 minutes. The etching solution described may comprise a solution of Enprep 250 at a temperature of 60°C.

The etched busbar 10 is then immersed or spray rinsed in demineralised water.

### Smut removal:

The busbar 10 is immersed in a smut removal solution for the removal of any residue cleaner/etcher solution and to ensure the busbar 10 surface material is 'active' for subsequent processes. The smut removal solution described may comprise a solution of Victa-D-Ox at room temperature.

The busbar 10 is then immersed or spray rinsed in demineralised water.

### Initial Zinc plating:

The portion 20 of the busbar 10 is immersed for a period of time in a zincating solution for depositing a zinc layer on the surface 13 of the busbar 10 for providing good adhesion with nickel in subsequent steps. Typically the busbar 10 will be immersed in the zincating solution for a period of around 2 minutes. The initial zincating solution described may comprise a solution of Bondal at a temperature of 30°C.

The busbar 10 is then immersed or spray rinsed in demineralised water.

The portion 20 of the busbar 10 is then immersed into a zincate strip solution for lightly etching the deposited zinc layer and for exposing areas on the surface 13 of the busbar 10 not yet completely covered by the deposited zinc. The zincate strip solution described may comprise a solution of Alprep 291 at a temperature of 30°C.

The busbar 10 is then immersed or spray rinsed in demineralised water.

### Final Zinc plating:

The portion 20 of the busbar 10 is immersed into a final zincate solution to complete the zinc layer which improves adherence between the busbar 10 surface 13 and a subsequent nickel sulphamate solution. It also limits the sacrificial nature of the aluminium material due to the position of metal on the galvanic scale. The final zincate solution described may comprise a solution of Bondal at a temperature of 30°C.

The busbar 10 is then immersed or spray rinsed in demineralised water.

### Nickel Electroplating:

The portion 20 of the busbar 10 is immersed with a live electrical charge into a bath of nickel sulphamate solution. A boric acid bath of 45g/l boric acid at a preferred temperature of around 50° C is required for this process. The actual operating conditions for depositing of the nickel may vary however the preferred embodiment applies approximately 200 amperes for each busbar 10 to achieve an electrodeposition of nickel onto the busbar 10 surface 13. The nickel coating preferably provides an insulating barrier 22 having a thickness of approximately 10 µm after a 10 to 15 minute period of time. The nickel sulphamate solution described may comprise a Barrett Sn solution.

Typically the nickel coating produces a semi-matte finish on the external surface 13 of a busbar 10. However it is found that this semi-matte finish marks easily through subsequent handling of the busbar 10.

### Further non-marking step

To overcome the problem of marking the semi-matte finish merely through handling a further non-marking step may be included in the method of the present invention. The further non-marking step comprises an additional immersion of a nickel plated busbar 10.

This further step is advantageously found to improve corrosion resistance of the busbar 10 and to limit marking of the nickel finish. Also, it has been advantageously found to improve the amount of adhesion between the insulating barrier 26 and the exterior surface 13.

The insulating barrier 26 manufactured in accordance with the present invention can provide over 96 hours of salt spray protection without changing the colour of the busbar 10 or effecting the resistance in a busbar 10 connection.

### Electrically Insulating Barrier

Seen in Figures 1 and 2 the busbar 10 manufactuared according to a preferred embodiment of the present invention comprises an electrically insulating barrier 26 disposed about the second portion 24 of the busbar 10. The insulating barrier 26 comprises a plastic surface coating 26 that is arranged to substantially cover at least a portion of the external surface 13 area as defined by the second portion 24. It is to be understood that the plastic surface coating 26 is configured to be substantially ductile and have substantially electrically insulating properties.

It should be understood that the electrically insulating barrier 26 may be equally effective for insulating a busbar 10 made from either aluminium or copper material. The plastic material used as the surface coating 26 comprises an epoxy thermoset material that provides a plastic surface coating 26 substantially covering the second portion 24 and which has sufficient ductibility to conform to the shape of the busbar 10 before, during and after shaping of the busbar without compromising the insulation properties of the barrier.

A method of providing a plastic surface coating on a busbar 10 in accordance with a preferred embodiment of the present invention is described below.

### Aluminium material busbars:

An aluminium busbar 10 is suspended on a mounting rack for pre-treatment and the powder coating processes.

A busbar 10 of aluminium material is immersed and/or spray rinsed in a demineralised water to remove any excess solution (remaining from the metallic surface coating process).

The portion 24 of the busbar is immersed and/or sprayed with a passivation solution to prevent marking as well as adding a layer that provides adhesion for the powder coating process described in the following steps. Typically this passivation solution is a water based lacquer such as Hydroclear at room temperature.

The busbar is then heated to around 60°C to harden the lacquer in preparation for handling and/or the subsequent powder coating process.

### Copper material busbars pre-treatment:

A busbar 10 of copper material is suspended on a mounting rack for pre-treatment and the powder-coating process.

The busbar 10 is immersed in cleaner solution (such as Hullclean 810 at 60°C) to ensure the copper surface 13 is clean and active for subsequent steps by removal of any soil/grease etc from the busbar 10 surface 13.

The busbar 10 is immersed and/or spray rinsed in a demineralised water to remove excess cleaner solution.

The busbar 10 is then immersed and/or sprayed with a solution to prevent marking as well as adding a layer that provides adhesion for the powder coating process described in the following. Typically this solution comprises a water based lacquer such as Hydroclear at room temperature.

The plastic surface coating 26 comprises a thermoset plastic material which is applied to the busbar 10 second portion 24 using powder coating surface treating techniques. Preferably the method of producing an insulating barrier 26 in accordance with the present invention uses a fluidised process comprising at least the following steps:

### Mounting:

The busbar 10 (of either aluminium or copper material) undergoing treatment is mounted on a jig or rack for improved handling and is then heated to around 180°C.

### Coating:

Once the busbar 10 is heated the portion 24 is immersed into a powder fluidised bed for around 5-8 seconds thereby providing the portion 24 of the busbar 10 with a coating of uncured powder.

### Curing:

The busbar 10, coated with the uncured powder, is then baked for around 30 minutes at a temperature of 150°C to cure the powder coating and achieve the plastic surface coating 26.

It should be understood that the plastic surface coating 26 provides an effective electrically insulating barrier which, in practice, complies with relevant standards, such as national AS/NZS standards or the IEC (International Electrotechnical Commission) equivalents. These standards set guidelines and rules in respect of desirable material properties with particular regard given to insulation resistance, flammability rating and temperature endurance for example.

Some further advantageous features of the insulating plastic surface coating 26 manufactured in accordance with the present invention are as follows:
- Lower cost of busbar 10 insulation when compared with known methods;
- The insulated busbars 10 can be cut, holes punched or drilled, and bent as required;
- Areas covered by the plastic surface coating 26 are selectively accessible by scoring and peeling the plastic surface coating 26 away from the busbar 10 thereby exposing the external surface 13 beneath;
- Provides greater durability than known heat shrink methods;
- Provides compact insulation with less impact on the dimensions of a busbar 10 than known PVC sleeving methods; and
- Tough, chip resistant, water resistant and provides improved corrosion protection.

The plastic surface coating 26 provides a busbar 10 that does not require additional time to be spent on fitting insulation materials to the switchboard or the busbar before or after installation of a busbar 10.

In general the quality of a powder coating is normally measured by the quality of adhesion with the base material and by the properties of hardness or durability of a coating. However it is to be understood that the present invention requires only that the plastic surface coating 26 has sufficient adhesion with the external surface 13 of portion 24 to remain in place on the busbar 10 during shaping and use of the busbar 10. When undergoing shaping as required for a particular switch board or other electrical distribution apparatus. The coating 26 is to be sufficiently ductile to avoid being compromised by fracturing, splitting or cracking for example when the busbar 10 is worked upon.

The plastic surface coating 26 in accordance with the present invention has sufficient ductile properties to permit a busbar 10 to be bent at an angle of 90° as seen in Figure 1 or more from beginning as a flat configuration shown in Figure 2, without compromising the insulating properties of the plastic surface coating 26 in any way.

Further, as shown in Figures 1 and 2 the plastic surface coating 26 is arranged to be of a suitable plasticity/ductility to enable at least a portion of the plastic surface coating 26 to be selectively peeled away from the surface of the busbar 10 as may be required to make a new connection for example. It is an advantage of the present invention that an area of the external surface 13 from which the plastic surface coating 26 has been removed remains clean and without any surface coating 26 residue.

In a preferred embodiment of the present invention the plastic surface coating 26 is applied subsequent to the application of the metallic surface coating 22.

In use, a busbar 10 manufactured in accordance with the present invention will be provided for commerce and to electrical distributors and the like. In one preferred embodiment a busbar 10 of aluminium material is provided having the metallic and plastic surface coatings 22, 26 thereon as described hereinbefore, or alternatively, a busbar 10 of copper material having a plastic surface coating 26 on a portion thereof may be provided. The busbar 10 will be available in all the industry standard sizes.

A user, such as a switch board designer or electrician for example can manipulate or shape the busbar 10 manufactured according to the present invention as required for any particular electrical distribution application as is known in the art. An advantage of the busbar 10 lies in the pre-insulated feature of the busbar 10 such that the user can shape and fit the busbar 10 without further concern or additional steps relating to insulating of the busbar 10.

After selecting a busbar 10 of suitable dimensions the user can proceed to fit the busbar 10 by shaping or bending the busbar 10 to suit the electrical apparatus or switch board dimensions. The busbar 10 can be further adapted by drilling holes for connection with other electrical components such as other busbars 10 or wiring for example as is known in the art. Where a position for a desired hole or connection is disposed in the second portion 24 and therefore covered by the plastic second surface coating 26 the coating 26 can be selectively removed from the area by suitable means, such as by marking the coating 26 with a scribe or similar tool and then manually peeling the plastic surface coating 26 away from the busbar 10 by hand, as indicated in Figure 2.

Once the busbar 10 has been adapted to conform to an electrical apparatus it may then be fitted in position by known means such as bolting or clamping. A contact lubricant may improve the performance of an electrical connection regardless of the type of metal used in a busbar, therefore it is envisaged that contact lubricants may be used with the present invention.

Modifications and variations as would be apparent to a skilled addressee are deemed to be within the scope of the present invention, as defined by the appending claims.

## Claims

1. A method for manufacturing a pre-insulated busbar (10), for use in the distribution of electricity, the pre-insulated busbar (10) comprising an electrically conductive metallic body (12) having an external surface (13) disposed between peripheral ends (6,8), and a substantially ductile electrically insulating barrier (26) of an epoxy thermoset material, wherein the insulating barrier (26) is disposed on the external surface (13) to overlay at least a portion (24) of the external surface (13) for substantially isolating the portion (24) underlying the insulating barrier (26) from an electrical contact, **characterised in that**,
the method comprises the steps of:
- providing an electrically conductive metallic body (12) having an external surface (13) disposed between peripheral ends (6,8);
- heating the metallic body (12) to a temperature between 140°C and 200°C;
- immersing at least a portion (24) of the heated metallic body (12) into a powder fluidized bed for a period of 3 to 10 seconds; and,
- baking the metallic body (12) at a temperature between 130°C and 170°C for a period of time greater than 20 minutes
such that the insulating barrier (26) has a structural integrity and insulating function that is maintained during a bending of the underlying portion (24) of the metallic body (12) through an angle up to 90°.

2. A method according to claim 1, **characterised in that** the portion 24 is immersed into the powder fluidized bed for a period of time, such that the insulating barrier 26 comprises a thickness greater than 0.02 mm.

3. A method according to claim 1 **characterised in that** the metallic body 12 is bent into an L shaped configuration.

4. A method according to any one of the preceding claims, **characterised in that**, the provided electrically conductive metallic body (12) is pretreated such that the metallic body 12 further comprises a conductive barrier 22 disposed about at least a portion 20 of the external surface 13, so that the conductive barrier 22 substantially limits a formation of a metallic oxide layer upon the metallic body 12.

5. A method according to claim 4, **characterised in that** the metallic body (12) is pretreated such that the conductive barrier 22 comprises a metallic surface coating 22.

6. A method according to claims 4 and 5, **characterised in that** the metallic body (12) is pretreated such that the conductive barrier 22 comprises a nickel material.

7. A method according to claims 1 and 6, **characterised in that** the provided metallic body 12 comprises an aluminium material.

8. A method according to claim 4, **characterised in that** the portion 20 substantially comprises the entire external surface 13.

9. A method according to claim 5, **characterised in that** the metallic surface coating 22 is formed to comprise a thickness between 0.5µm to 15µm.

10. A method according to claim 4, **characterised in that** the portion 20 and the portion 24 overlay one another.

## Patentansprüche

1. Verfahren zur Herstellung einer vorisolierten Sammelschiene (10) zur Verwendung bei der Verteilung von Elektrizität, wobei die vorisolierte Sammelschiene (10) einen elektrisch leitenden Metallkörper (12), der eine zwischen peripheren Enden (6, 8) angeordneten Außenfläche (13) aufweist, und eine im Wesentlichen duktile elektrisch isolierende Barriere (26) aus einem wärmehärtenden Epoxidmaterial umfasst, wobei die isolierende Barriere (26) auf der äußeren Oberfläche (13) angeordnet ist, um mindestens einen Teil (24) der äußeren Oberfläche (13) zu überlagern, um den unter der isolierenden Barriere (26) liegenden Teil (24) im Wesentlichen von einem elektrischen Kontakt zu isolieren, **dadurch gekennzeichnet, dass**
das Verfahren die folgenden Schritte umfasst:
- Bereitstellen eines elektrisch leitfähigen Metallkörpers (12), der eine Außenfläche (13) aufweist, die zwischen peripheren Enden (6, 8) angeordnet ist;
- Erwärmen des Metallkörpers (12) auf eine Temperatur zwischen 140 °C und 200 °C;
- Eintauchen mindestens eines Abschnitts (24) des erwärmten Metallkörpers (12) in ein Pulverwirbelbett über einen Zeitraum von 3 bis 10 Sekunden; und
- Einbrennen des Metallkörpers (12) bei einer Temperatur zwischen 130 °C und 170 °C über einen Zeitraum von mehr als 20 Minuten,
so dass die isolierende Barriere (26) eine strukturelle Integrität und isolierende Funktion aufweist, die während eines Biegens des darunter liegenden Abschnitts (24) des Metallkörpers (12) um einen Winkel bis zu 90° aufrechterhalten wird.

2. Verfahren nach Anspruch 1, **dadurch gekennzeichnet, dass** der Abschnitt (24) über einen solchen Zeitraum in das Pulverwirbelbett eingetaucht wird, sodass die isolierende Barriere (26) eine Dicke von mehr als 0,02 mm aufweist.

3. Verfahren nach Anspruch 1, **dadurch gekennzeichnet, dass** der Metallkörper (12) in eine L-förmige Konfiguration gebogen wird.

4. Verfahren nach einem der vorstehenden Ansprüche, **dadurch gekennzeichnet, dass** der bereitgestellte elektrisch leitende Metallkörper (12) so vorbehandelt wird, dass der Metallkörper (12) weiter eine leitende Barriere (22) umfasst, die um mindestens einen Abschnitt (20) der Außenfläche (13) herum angeordnet ist, so dass die leitende Barriere (22) eine Bildung einer Metalloxidschicht auf dem Metallkörper (12) im Wesentlichen begrenzt.

5. Verfahren nach Anspruch 4, **dadurch gekennzeichnet, dass** der Metallkörper (12) so vorbehandelt wird, dass die leitende Barriere (22) eine metallische Oberflächenbeschichtung (22) umfasst.

6. Verfahren nach den Ansprüchen 4 und 5, **dadurch gekennzeichnet, dass** der Metallkörper (12) so vorbehandelt wird, dass die leitende Barriere (22) ein Nickelmaterial umfasst.

7. Verfahren nach den Ansprüchen 1 und 6, **dadurch gekennzeichnet, dass** der bereitgestellte Metallkörper (12) ein Aluminiummaterial umfasst.

8. Verfahren nach Anspruch 4, **dadurch gekennzeichnet, dass** der Abschnitt (20) im Wesentlichen die gesamte Außenfläche (13) umfasst.

9. Verfahren nach Anspruch 5, **dadurch gekennzeichnet, dass** die metallische Oberflächenbeschichtung (22) so geformt wird, dass sie eine Dicke von 0,5 µm bis 15 µm umfasst.

10. Verfahren nach Anspruch 4, **dadurch gekennzeichnet, dass** der Abschnitt (20) und der Abschnitt (24) einander überlagern.

## Revendications

1. Procédé de fabrication d'une barre omnibus pré-isolée (10), destinée à servir dans la distribution d'électricité, la barre omnibus pré-isolée (10) comprenant un corps métallique électriquement conducteur (12) ayant une surface externe (13) disposée entre des extrémités périphériques (6,8), et une barrière électriquement isolante sensiblement ductile (26) en un matériau époxy thermodurci, dans lequel la barrière isolante (26) est disposée sur la surface externe (13) pour recouvrir au moins une partie (24) de la surface externe (13) afin d'isoler sensiblement la partie (24) sous-jacente à la barrière isolante (26) contre un contact électrique, **caractérisé en ce que**
le procédé comprend les étapes consistant à :
- fournir un corps métallique électriquement conducteur (12) ayant une surface externe (13) disposée entre des extrémités périphériques (6,8) ;
- chauffer le corps métallique (12) à une température comprise entre 140 °C et 200 °C ;
- plonger au moins une partie (24) du corps métallique chauffé (12) dans un lit fluidisé de poudre pendant une durée de 3 à 10 secondes ; et
- cuire le corps métallique (12) à une température comprise entre 130 °C et 170 °C pendant une durée supérieure à 20 minutes
de telle sorte que la barrière isolante (26) a une intégrité structurelle et une fonction isolante qui est conservée lors d'un pliage de la partie sous-jacente (24) du corps métallique (12) sur un angle allant jusqu'à 90°.

2. Procédé selon la revendication 1, **caractérisé en ce que** la partie (24) est plongée dans le lit fluidisé de poudre pendant une durée telle que la barrière isolante (26) comprend une épaisseur supérieure à 0,02 mm.

3. Procédé selon la revendication 1, **caractérisé en ce que** le corps métallique (12) est plié selon une configuration en forme de L.

4. Procédé selon l'une quelconque des revendications précédentes, **caractérisé en ce que** le corps métallique électriquement conducteur (12) fourni est prétraité de telle façon que le corps métallique (12) comprend en outre une barrière conductrice (22) disposée autour d'au moins une partie (20) de la surface externe (13), de telle sorte que la barrière conductrice (22) limite sensiblement une formation d'une couche d'oxyde métallique sur le corps métallique (12).

5. Procédé selon la revendication 4, **caractérisé en ce que** le corps métallique (12) est prétraité de telle façon que la barrière conductrice (22) comprend un revêtement de surface métallique (22).

6. Procédé selon les revendications 4 et 5, **caractérisé en ce que** le corps métallique (12) est prétraité de telle façon que la barrière conductrice (22) comprend un matériau en nickel.

7. Procédé selon les revendications 1 et 6, **caractérisé en ce que** le corps métallique (12) fourni comprend un matériau en aluminium.

8. Procédé selon la revendication 4, **caractérisé en ce que** la partie (20) comprend sensiblement l'ensemble de la surface externe (13).

9. Procédé selon la revendication 5, **caractérisé en ce que** le revêtement de surface métallique (22) est formé pour comprendre une épaisseur entre 0,5 µm et 15 µm.

10. Procédé selon la revendication 4, **caractérisé en ce que** la partie (20) et la partie (24) sont superposées l'une sur l'autre.
